

[54] COLOR ELECTROPHOTOGRAPHIC PROCESS USING PHOTOCONDUCTIVE PARTICLES IN LIQUID DEVELOPER

[75] Inventors: Masamichi Sato; Hajime Miyazuka, both of Asaka, Japan

[73] Assignee: Xerox Corporation, Stamford, Conn.

[22] Filed: Nov. 13, 1974

[21] Appl. No.: 523,612

**Related U.S. Application Data**

[62] Division of Ser. No. 887,980, Dec. 24, 1969, abandoned.

[30] **Foreign Application Priority Data**

Dec. 28, 1968 Japan ..... 44-980

[52] U.S. Cl. ..... 96/1.2; 252/62.1 L; 96/1 LY

[51] Int. Cl.<sup>2</sup> ..... G03G 5/12; G03G 13/01; G03G 9/00

[58] Field of Search ..... 96/1.2, 1 LY; 252/62.1

[56]

**References Cited**

**UNITED STATES PATENTS**

|           |         |                      |           |
|-----------|---------|----------------------|-----------|
| 3,076,722 | 2/1963  | Greig .....          | 96/1.2    |
| 3,079,272 | 2/1963  | Greig .....          | 117/37 LE |
| 3,150,976 | 9/1964  | Johnson .....        | 252/62.1  |
| 3,220,830 | 11/1965 | Kashiwabara .....    | 252/62.1  |
| 3,276,896 | 12/1966 | Fisher .....         | 96/1 LY   |
| 3,293,183 | 12/1961 | Matkan .....         | 252/62.1  |
| 3,357,830 | 12/1967 | Bixby .....          | 96/1.2    |
| 3,403,023 | 9/1968  | Carrington .....     | 96/1.7    |
| 3,703,370 | 11/1972 | Sugarman et al. .... | 252/62.1  |

Primary Examiner—Jack P. Brammer

[57]

**ABSTRACT**

Reproduction of a multicolor original is obtained in an electrophotographic process with multiple development employing a liquid developer comprising an insulating liquid and suspended therein photoconductive particles and colored toner particles. Prior to the second and subsequent development steps, the imaging surface is contacted with a toner free insulating liquid.

**11 Claims, 6 Drawing Figures**





FIG. 1



FIG. 2A



FIG. 2B

INVENTORS  
MASAMICHI SATO  
HAJIME MIYAZUKA  
BY

*Samuel S. Mott*  
ATTORNEY



FIG. 3



FIG. 4



FIG. 5

**COLOR ELECTROPHOTOGRAPHIC PROCESS  
USING PHOTOCONDUCTIVE PARTICLES IN  
LIQUID DEVELOPER**

This application is a divisional application of application Ser. No. 887,980, filed on Dec. 24, 1969, now abandoned.

**BACKGROUND OF THE INVENTION**

This invention relates to imaging systems and more particularly to liquid development systems and liquid developers for use in color reproduction utilizing multiple development.

Color electrophotography with multiple development is capable of producing color reproductions by the following exemplary procedures. A suitable photoconductor such as substantially white zinc oxide photosensitive paper, Electrofax paper for example, is electrostatically uniformly charged in the dark and then exposed through a green filter to an imagewise projection of a color image to form an electrostatic latent image on the photoconductor. The electrostatic latent image is then developed with magenta colored toner to form a magenta colored image corresponding to said electrostatic latent image. The zinc oxide photosensitive paper is again electrostatically uniformly charged in the dark and then exposed through a red filter to an imagewise projection of a colored image in register with said magenta developed image to form a second electrostatic latent image, which second image is developed with cyan colored toner. Similarly, the zinc oxide photosensitive paper is again electrostatically uniformly charged in the dark and then exposed through a blue filter to an imagewise projection of a colored image in register with said magenta and cyan developed images to form a third electrostatic latent image, which is then developed with yellow toner to complete a reproduced color image.

The sequence of exposures through colored filters in this multiple development process may be performed in any suitable sequence other than the green, red and blue sequence recited above.

A significant drawback of this multiple development process is that after the formation of the image of the first color and during the second imaging sequence consisting of uniformly charging and imagewise exposing followed by development with toner of the second color, the zinc oxide photosensitive paper is apt to be electrostatically charged more strongly in the portion where said first colored image is formed in comparison with the other portion where such image does not exist. In addition, the portion of the zinc oxide paper where the first colored image is formed is apt to retain charge in nonimage areas when imagewise exposed to a light pattern which is capable of neutralizing the electrostatic charge in the latter portion. This retained potential, which usually ranges from several volts to several tens of volts, arises from the fact that the ion absorbed by the toner during charging is not neutralized during the imagewise exposure to light. Since the toner usually consists of electrically insulating material the neutralization of the ion for example, held by the toner layer, for material the corona ion generated by corona discharge is hindered. Electroconductive toner cannot be employed in electrophotography with multiple development since the portion of the photoconductor having such toner on its surface during the second and third imaging sequences cannot bear electrostatic charge.

Furthermore, when the electrostatic charge on the first toner layer is not completely neutralized, the toner of second color tends to be improperly deposited onto the first toner layer, giving rise to impure color formation. Similar difficulties also arise in the development with the toner of the third color, and the tendency for improper toner deposition increases as the reflective optical density of the toner image already present is increased. The result of these characteristics is that it is very difficult to obtain color reproduction of satisfactory quality.

These difficulties have been lessened to some degree by the use of the techniques and materials disclosed in U.S. Pat. 3,060,020 which is herein incorporated by reference. Essentially therein disclosed is a technique utilizing toner chiefly consisting of photoconductive zinc oxide powder in order to provide appropriate photoconductive property to the toner image. This technique may be more fully understood by reference to FIGS. 1, 2A and 2B of the accompanying drawing in which:

FIG. 1 is an enlarged cross section of the toner particles.

FIG. 2A is an enlarged cross section of a toner image on an imaging surface.

FIG. 2B is an enlarged cross section of a fused toner image on an imaging surface.

In FIG. 1, toner particle 10 consists of core 11 composed of photoconductive zinc oxide particle surrounded by a colored resin layer 13, which may be composed either of pigment particles 12 dispersed in resin as shown or of resin colored with an appropriate dye. The resin 13 is required to be liquified by heat, and the melting point thereof is usually required to lie between about 90° and about 250° C. In addition, the resin layer is required to be highly insulating and to have sufficient capability to generate favorable frictional electricity (i.e. a capability to generate sufficiently strong positive charge if the latent image is negative). Furthermore the resin 13, when melted, should be of sufficiently low viscosity, preferably between about 45 and about 10,000 centipoises, so as to be removed from the surface of the zinc oxide core.

FIGS. 2A and 2B show the method of using the dry powder toner described in said U.S. Pat. in a dry development system. As shown in FIG. 2A, the toner image 21 is formed by toner particles 10 held onto the imaging surface 22 bearing an electrostatic latent image. The toner layer thus formed simply by means of electrostatic forces of attraction does not possess photoconductivity due to the high electric resistance of resin layer 13 surrounding the zinc oxide core 11. When the toner is melted by heat as shown in FIG. 2B, the resin 13 together with pigment 12 is spread onto the imaging surface thereby exposing the surface of zinc oxide core particle. As a result, the fixed toner layer 21' shown in FIG. 2B acquires photoconductive property on account of the exposed zinc oxide particles 11.

This process, however, has several drawbacks among which are the fact that the heating up to 90° - 250° C. required for melting the toner image may cause irreversible dilatation of the imaging surface which may result in the formation of unsatisfactory prints due to imperfect registration during the second and third imaging sequences. This difficulty is especially pronounced when the support material consists of paper, as for example in Electrofax paper. In addition, the colors obtained by this process are not of high satura-

tion but rather become whitish since the white zinc oxide powder is almost exposed to the surface after fixing of the toner image by heat. This difficulty results in impure color or lack of color density when three color images are superimposed one upon the other. The melting point and limited viscosity range of the resin seriously confine the selection of suitable materials to only certain types which also must be highly insulating and capable of being triboelectrically charged to a suitable polarity and potential. Furthermore, this dry developer toner cannot be used with a particle size smaller than a certain limit, and therefore is not capable of providing high resolution and satisfactory tone reproduction. Actually, the toner is frequently composed of aggregate of several to several tens of zinc oxide particles instead of being composed of a single particle as shown in the ideal case of FIG. 1.

#### SUMMARY OF THE INVENTION

It is therefore an object of this invention to provide a novel liquid developer.

It is another object of this invention to provide a novel liquid developer for use in color electrophotography with multiple development.

It is another object of this invention to provide a liquid developer containing photoconductive particles.

It is another object of this invention to provide a novel imaging system.

It is another object of this invention to provide an imaging system capable of high resolution and high color density.

It is another object of this invention to provide a color electrophotographic process capable of yielding color reproductions of improved quality.

It is another object of this invention to provide a color electrophotographic process with multiple development wherein the toner particles do not have to be fused to the imaging surface.

The above objects and others are accomplished generally speaking by providing an imaging system employing a liquid developer comprising a suspension in an insulating liquid of colored particles and white or dye sensitized photoconductive particles preferably in the presence of a dissolved or dispersed resin or oil for regulating the electrostatic charge or for stabilizing the suspension. In the liquid development technique with multiple development the surface bearing the electrostatic latent image after the development step of the first imaging sequence has been completed is subjected before contacting with the developer of the next imaging sequence to a step of pre-bathing in which said image bearing surface is brought into contact with a highly insulating liquid not containing toner in order to neutralize the electrostatic charge remaining in the toner layer from the development step of the previous imaging sequence to thereby prevent fogging of the several toner images. The pre-bathing step may be accomplished immediately after the development step or it may be accomplished prior to the development step in the second and third imaging sequences or it may be accomplished prior to the second and third exposure steps.

The invention may be more fully understood by reference to FIGS. 3, 4 and 5 of the accompanying drawing in which:

FIG. 3 is an enlarged cross section of the toner and photoconductive particles of this invention.

FIG. 4 is a cross section of a developed image formed by development with the liquid developer of this invention.

FIG. 5 is a graph showing the change in electrostatic charge on the toner image of FIG. 2.

The developer of this invention comprises toner particles and photoconductive particles suspended in an insulating liquid. The solids of the developer, generally represented in cross section in FIG. 3, comprise photoconductive particle 37, preferably consisting of particulate photoconductive material 33 and thin layer of resin 32 absorbed therearound.

The resin layer 32 is required to be as thin as possible to facilitate adequate exposure of photoconductive material 33 to dissipate any charge thereon. Otherwise, it would be necessary to employ some means to remove the resin layer to expose photoconductive particle 33. As disclosed in the following examples to provide adequate exposure, the resin covering the photoconductive particles is preferably soluble in the carrier liquid of the liquid developer. The resin layer may be employed in any suitable amount. Typically, the dispersed particle usually contains not more than about 2 parts by weight of the resin in 100 parts of particulate photoconductive material.

20 The photoconductive properties of the particle are hardly affected by the presence of this amount of resin and the electrostatic charge on the developed toner layer containing said particles is capable of being completely neutralized without the troublesome additional steps of removing the resin layer as indicated in the aforementioned U.S. Patent. Any suitable resin may be employed to provide a thin layer on a suitable particulate photoconductive material. Typical well known particulate photoconductive materials 25 include zinc oxide, zinc sulfide, cadmium sulfide, zinc selenide, cadmium selenide, titanium dioxide, zinc cadmium sulfide, zinc magnesium oxide, phthalocyanine, and polyvinyl carbazole. Typical resins that may be employed to provide the resin layer include epoxy ester resin, silicone resin, alkyd resin, phenol-formaldehyde resin, xylene-formaldehyde resin etc.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 99

Hansa yellow. When the colorant is an organic dye it is preferably insoluble in the carrier liquid and since the specific gravities of usual organic dyes and typical photoconductors such as zinc oxide are from about 1.5 to about 2 and about 5.6 respectively, the above weight ratio can be converted into 1.3 - 3500 parts by volume of zinc oxide particles 33 with respect to 100 parts by volume of dye particles 36, with the amount of resin 32 and 35 around the core particles 33 and 36 being neglected. Zinc oxide present in excess of this range will result in unfavorable color reproduction whereas the toner layer will show insufficient photoconductivity if the amount of zinc oxide does not reach this range.

Any suitable well known insulating liquid may be employed as the vehicle for the photoconductive particles and toner particles. Typical well known materials have volume resistivities greater than about  $10^{10}$  ohm-cm so as not to affect the electrostatic charge pattern on the insulating layer and low dielectric constants of less than about 3.4. Typical specific vehicles include among others, the nonpolar hydrocarbons and hydrocarbon derivatives such as benzene, kerosene, cyclohexane, toluene and carbon tetrachloride.

In FIG. 2A, the toner layer shows high electric resistance as the layer is composed of toner particles 10 electrically insulated from each other, whereas in FIG. 4 the electric carrier formed by the effect of light in the photoconductive particles 37 can easily unite with ions on toner particles present in the proximity of said particles 37 due to the uniform distribution of photoconductive particles 37 and toner particles 34 and the smaller distance between said photoconductive particles 37. Consequently, in the process of this invention, it is completely unnecessary to melt the toner layer by heat to expose the photoconductive particles. The present invention differs from the technique described with respect to FIGS. 1 and 2 in that the electrostatic charge remaining on the developed toner layer can be completely neutralized prior to development in the second or third development step simply by contacting said layer with an insulating liquid. In the liquid development technique with multiple development the image bearing surface after the first development step has been completed is subjected before contacting with the developer of the next development step to a step of pre-bathing in which said surface is brought into contact with a highly insulating liquid not containing toner in order to neutralize the electrostatic charge still remaining in the toner layer from the previous development sequence. The sequence of steps in this multiple development technique may include initial charging and exposure of the photoconductor through a suitable first filter followed by development with the appropriately colored liquid developer of this invention. The photoconductor with the first developed toner image thereon is subjected to the pre-bathing technique of this invention prior to the second imaging sequence comprising charging, exposing through an appropriate filter and developing with the corresponding colored liquid developer. After this second development sequence the photoconductor bearing the first and second development toner image is subjected to an additional pre-bathing technique prior to the development step of the third imaging sequence. While the above technique describes the pre-bathing step as the initial step in the second and third imaging sequence, it is necessary only that the photoconductor be subjected to the pre-bathing technique prior to the development

step in the second and third imaging sequence. In this manner, any residual charge remaining on the imaging surface from a prior imaging sequence is effectively neutralized prior to subsequent deposition of toner in response to an electrostatic charge pattern. Therefore, toner is electrostatically attracted to only the image areas produced in each imaging sequence and is not deposited on the photoconductor in response to more than one or overlapping image areas of several imaging sequences. To provide this result, the photoconductor may be subjected to the pre-bathing treatment prior to charging, exposure or development in the second and third imaging sequence.

During uniform electrostatic charging in the dark the zinc oxide photosensitive paper as shown in the toner layer depicted in FIG. 4 is electrostatically charged by the adsorption of ions. As shown in FIG. 5, the surface potential of toner layer reaches  $V_1$  by means of electrostatic charging such as by corona discharge carried out for a period between time 0 and  $t_1$  in the dark, and then decreases to  $V_2$  by interrupting said charging at time  $t_1$  and effecting imagewise exposure from time  $t_1$  to  $t_2$ . The proportion of photoconductive particles 37 is preferably as small as possible since a larger proportion thereof will inevitably result in the deterioration of color quality although a larger portion will enable the attainment of a lower value of  $V_2$  against a determined amount of light of exposure. Successively the surface potential can be rapidly reduced to zero by bringing the toner image into contact with the pre-bath liquid. This neutralization of surface potential by pre-bath step provides a great advantage of this invention in comparison with the process of aforesaid U.S. Patent. The neutralization by means of the pre-bath step can be explained by the formation of ions by the triboelectric contact between the particles and pre-bath liquid, and also by the fact that the liquid filling the gap between the particles gives mobility to the ions.

An additional advantage of this invention lies in the fact that the ratio between the amounts of pigment particles 34 and photoconductive particles 37 can be arbitrarily varied during or prior to use of the developer, whereas in the process disclosed in U.S. Patent this ratio is fixed when the developer is prepared. When reproducing colored positive image from a colored positive original pattern onto a panchromatically sensitized photosensitive layer by means of the multiple development process, it is necessary to select the order of development in order to minimize the effect of undesirable spectral absorption of available dyes or pigments of cyan, magenta and yellow. Since these dyes and pigments generally show undesirable spectral absorption in the shorter wavelength side with respect to the main absorption region thereof, it is preferred to provide development in the order of shorter to longer wavelength region with respect to the main absorption of these dyes or pigments, namely in the order of yellow, magenta and cyan successively. At this point it is to be noted that yellow-colored dyes or pigments generally have tendency to show relatively high retentive potential. Consequently, the process of this invention is particularly effective when applied in the liquid developer containing yellow dye or pigment, and is capable of providing almost ideal color reproduction.

#### DESCRIPTION OF PREFERRED EMBODIMENTS

The following preferred examples further define, describe and compare preferred materials, methods

and techniques of the present invention. In the examples, all parts and percentages are by weight unless otherwise specified.

### EXAMPLE I

A yellow developer is prepared by dispersing the following material by means of ultrasonic wave of 29 KC and 150 W to produce Solution A.

|                        |                       |
|------------------------|-----------------------|
| Benzidine yellow       | 0.4 parts by weight   |
| Styrenated-alkyd resin | 0.5 parts by weight   |
| Linseed oil            | 0.1 parts by weight   |
| Cyclohexane            | 400.0 parts by weight |
| Kerosene               | 100.0 parts by weight |

The following materials are dispersed by means of ultrasonic wave of 29 KC and 150 W to form Solution B:

|                            |                       |
|----------------------------|-----------------------|
| Photoconductive zinc oxide | 0.1 part by weight    |
| Styrenated-alkyd resin     | 0.5 part by weight    |
| Linseed oil                | 0.1 part by weight    |
| Cyclohexane                | 400.0 parts by weight |
| Kerosene                   | 100.0 parts by weight |

The developer of this invention may be prepared by mixing Solution A and Solution B in a suitable ratio. The following table shows the values of  $V_1$  and  $V_2$  for various mixing ratios, wherein  $t_1$  and  $t_2$  are 10 and 20 seconds respectively, and the photosensitive material is exposed to white light of 400 lux at  $t = t_1$  and is brought into contact with kerosene at  $t = t_2$ .

| No.        | 1     | 2  | 3  | 4  | 5  |
|------------|-------|----|----|----|----|
| Solution A | 100CC | 50 | 30 | 25 | 20 |
| Solution B | 0CC   | 50 | 70 | 75 | 80 |
| $V_1$      | 27V   | 35 | 32 | 25 | 20 |
| $V_2$      | 25V   | 25 | 19 | 13 | 13 |
| $V_3$      | 7V    | 0  | 0  | 0  | 0  |

As can be seen from the above table, the value of  $V_3$  remains at 7 volts when photoconductive particles are not dispersed in the developer, leading to impure color due to the improper attraction of other toner in the succeeding development to these charged toner areas.

On the other hand, the presence of photoconductive particles in an appropriate amount effectively reduces the value of  $V_3$  to zero, and still the whitening of the yellow image obtained due to the adhering of the white zinc oxide particles is hardly observable in the images developed with the developers 2 through 5.

Although the Solution A and Solution B are prepared in diluted state at first in this example, it is also possible to prepare the developer by preparing a paste with linseed oil, zinc oxide powder and resin and then dispersing the paste into dispersion media such as cyclohexane or kerosene directly prior to use.

### EXAMPLE II

The following materials are blended in a ball mill for one hour to give Paste A:

|                                                                                                      |                    |
|------------------------------------------------------------------------------------------------------|--------------------|
| Brilliant carmine 6B                                                                                 | 30 parts by weight |
| Varnish obtained by heating 1:1 mixture of linseed oil and rosin denatured phenol-formaldehyde resin | 60 parts by weight |

-continued

Linseed oil 10 parts by weight

In a similar manner, Paste B is prepared of the following materials:

|                            |                    |
|----------------------------|--------------------|
| Photoconductive zinc oxide | 20 parts by weight |
| Varnish                    | 60 parts by weight |
| Linseed oil                | 20 parts by weight |

A developer obtained by dispersing about 1 gram of Paste A in 800 CC of cyclohexane and 200 CC of kerosene provides a developed toner image having a reflective optical density of about 2.0 and  $V_1$  and  $V_3$  are found to be 8 and 3 volts respectively. On the other hand,  $V_3$  is found to be zero in the toner images developed in the same manner with a developer obtained by dispersing from about 0.1 to about 2.0g of Paste B into the above-mentioned developer. The whitening of obtained image due to dispersed zinc oxide powder is hardly observable.

### EXAMPLE III

A cyan developer is prepared by blending the following materials in a ball mill for one hour to form Paste A:

|              |                    |
|--------------|--------------------|
| Millary blue | 40 parts by weight |
| Varnish      | 50 parts by weight |
| Linseed oil  | 10 parts by weight |

Paste B is also prepared similarly from the following materials:

|                            |                    |
|----------------------------|--------------------|
| Photoconductive zinc oxide | 20 parts by weight |
| Varnish                    | 60 parts by weight |
| Linseed oil                | 20 parts by weight |

A developer prepared by dispersing 1 gram of Paste A in 800 CC of cyclohexane and 200 CC of kerosene provides a developed toner image having a reflective optical density of about 2.0 and  $V_1$  and  $V_3$  are found to be 3 and 2 volts respectively. On the other hand,  $V_3$  is reduced to zero in similar toner images developed by developers prepared by dispersing from about 0.05 to about 2.0g of Paste B into the above-mentioned developer.

### EXAMPLE IV

A yellow developer is prepared by the procedure of Example I except that the white photoconductive zinc oxide powder in Example I is replaced by pale yellow dye-sensitized zinc oxide powder, which has been prepared by placing the zinc oxide particles in the following composition for sufficient time to cause absorption of dye onto the zinc oxide particles.

|                                         |              |
|-----------------------------------------|--------------|
| White photoconductive zinc oxide powder | 10 grams     |
| Titanium yellow                         | 3 milligrams |
| Methanol                                | 40 CC        |

The zinc oxide particles are then separated by filtration and dried. The sensitized zinc oxide thus obtained increases the photographic sensitivity of the developer

for white light more than 10 times, exhibits a lower value of  $V_2$  due to its pale yellow color, and further improves the color of toner itself. Sensitization with other sensitizing dyes can be carried out in a similar manner.

The developers disclosed in Examples I through IV are suitable for exposure with white light through a color separation negative image and are not suitable for exposure directly from the colored original through a color separation filter.

The following example provides a developer capable of use with direct exposure from a colored original through a color separation filter.

#### EXAMPLE V

A yellow developer is prepared by dispersing the following materials by means of ultrasonic wave for 10 minutes to obtain Solution A:

|                  |                     |
|------------------|---------------------|
| Benzidine yellow | 0.4 parts by weight |
| Varnish          | 0.4 parts by weight |
| Linseed oil      | 0.1 parts by weight |
| Cyclohexane      | 800.0 CC            |
| Kerosene         | 200.0 CC            |

Similarly the following materials are dispersed by means of ultrasonic wave for 10 minutes to obtain Solution B:

|                              |                     |
|------------------------------|---------------------|
| Dye-sensitized<br>zinc oxide | 0.2 parts by weight |
| Varnish                      | 0.5 parts by weight |
| Linseed oil                  | 0.1 parts by weight |
| Cyclohexane                  | 800 CC              |
| Kerosene                     | 200 CC              |

The liquid developer is prepared by mixing about equal parts of Solution A and Solution B. The dye sensitized zinc oxide is prepared by stirring 10g of photoconductive white zinc oxide powder having a particle size of from about 0.1 to about 0.5 micron in a solution of the following formulation.

|                    |       |
|--------------------|-------|
| Rhodamin B         | 3 mg  |
| Brilliant blue FCF | 3 mg  |
| Methanol           | 40 CC |

After 30 minutes the absorption of sensitizing dyes by the zinc oxide powder, is terminated by separating the zinc oxide particles by centrifuging and drying the separated zinc oxide particles. The zinc oxide particles obtained are dyed a blue color and therefore stand in a complementary relationship with yellow. Generally, if the zinc oxide is dye-sensitized for a color (generally the color of light absorbed by the colored particle) standing in complementary relationship with the color of particle (yellow in this example), then the toner image obtained by the first development shows photoconductivity against light of wavelength region employed in the second and third exposure through appropriate color separation filters. In this example, zinc oxide particles having absorbed blue dyes are capable of showing photoconductivity against green and red light.

In a similar manner, it is necessary to carry out the dye-sensitization of zinc oxide with green dye when the first development is to be effected with magenta toner, or with red dye when the first development is to be effected with cyan toner.

Furthermore, when the first and second developments are to be carried out respectively with yellow and magenta toner, then the zinc oxide contained in the second toner should be sensitized with a dye having a color capable of absorbing red light such as cyan, blue or green since the third exposure should necessarily be carried out with red light. Photoconductivity is not required for the toner used in the third development sequence.

- 10 The generalization of this Example V leads to the fact that the first color developer should be a highly insulating liquid in which are suspended particles of said first color and photoconductive zinc oxide particles sensitized with dye so as to show photoconductivity to the wavelength region of light reflected from said first colored particles and that the second color developer should be a highly insulating liquid in which suspended are particles of a second color and photoconductive zinc oxide particles sensitized with dye so as to show 15 photoconductivity to the wavelength region of light which is reflected by both the particles of the first color and the second color.

#### EXAMPLE VI

- 20 A commercially available photoconductive insulating sheet comprising white zinc oxide in an insulating film-forming binder on a paper backing is negatively charged in conventional manner and is exposed to a colored original through a blue filter. The electrostatic latent image is developed with the liquid developer described in Example V by immersing the zinc oxide sheet in a bath of the developer. The zinc oxide sheet is then charged in conventional manner and exposed while in registration with the position during the first 25 exposure to the same colored original through a green filter. The zinc oxide sheet is uniformly contacted with kerosene by immersing it in a bath of kerosene. The second electrostatic latent image on the zinc oxide sheet is then developed by immersing the sheet in a bath of the liquid developer described in Example II except that the zinc oxide has been dye sensitized with brilliant green in a manner similar to the dye sensitization described in Example V. The zinc oxide sheet is again charged and exposed while in registration with the position during the first and second exposures to the same color original through a red filter. The zinc oxide sheet is then immersed in a bath of kerosene. The third electrostatic latent image on the zinc oxide sheet is then developed by contacting it with a dispersion of 30 about one gram of Paste A of Example III in 800 cubic centimeters of cyclohexane and 200 cubic centimeters of kerosene. The resulting color reproduction when compared to the original is a faithful reproduction of the several color image areas with good color density and with substantially no background.

35 It is readily realized from the foregoing discussion and exemplary embodiments that the developer and processes of this invention provide superior and unique reproducing capabilities. The developers of this invention enable the reproduction of multicolor originals with exceptional accuracy and substantially no undesirable overlapping of colors by forming two or more color coded electrostatic latent images and developing the images with a developer having toner particles of complementary color. The color coded electrostatic latent images may be created by the use of color separation negative images or exposure directly through a filter and thereby enables exposure of the photocon-

ductor to light of a selected wavelength. The development of electrostatic latent images coded in response to wavelength of light corresponding to the primary colors with the liquid developers of this invention enables the reproduction of multicolor images without the necessity of a toner fusing step and since finer size particulate material may be employed produces reproductions of superior quality.

Although specific materials and operational techniques are set forth in the above exemplary embodiments using the developer composition and development techniques of this invention, these are merely intended as illustrations of the present invention. There are other developer materials and techniques than those listed above which may be substituted for those in the examples with similar results.

Other modifications of the present invention will occur to those skilled in the art upon a reading of the present disclosure which modifications are intended to be included within the scope of this invention.

What is claimed is:

1. The method of producing a multicolor reproduction of an original colored object comprising the steps of:

- a. charging a photoconductive insulating layer;
- b. exposing the charged layer to said original colored object through a colored filter to form a first primary color coded electrostatic latent image on said layer;
- c. developing said first electrostatic latent image with a liquid developer having a color complementary to said first color coded latent image, said liquid developer comprising a carrier liquid having a dielectric constant of less than about 3.4 and a volume resistivity of greater than about  $10^{10}$  ohm-cm so as not to affect an electrostatic latent image formed on an insulating layer, and dispersed in said carrier liquid, a mixture of discrete colored toner particles and discrete photoconductive particles, said colored toner particles substantially lacking the property of photoconductivity and comprising a colorant selected from the group consisting of a pigment and a dye having a thin layer of a resin absorbed therearound, said photoconductive particles comprising particulate photoconductive material having a thin layer of a resin absorbed therearound, said thin layer of said resin absorbed therearound said particulate photoconductive material being sufficiently thin to facilitate exposure of said particulate photoconductive material and dissipate any charge thereon, said photoconductive particles being present in an amount of from about 5 to about 104 parts by weight for every 100 parts by weight of said colored toner particles;
- d. contacting said photoconductive insulating layer with an insulating liquid other than the developer liquid to neutralize any residual charge in the portion of said layer developed in step (c);
- e. charging said photoconductive insulating layer;
- f. exposing the charged layer to said original colored object through a colored filter to form a second primary color coded electrostatic latent image on said layer;
- g. developing said second electrostatic latent image with a liquid developer having a color complementary to said second color coded image; said liquid developer comprising a carrier liquid having a dielectric constant of less than about 3.4 and a volume

resistivity of greater than about  $10^{10}$  ohm-cm so as not to affect an electrostatic latent image formed on an insulating layer, and dispersed in said carrier liquid, a mixture of discrete colored toner particles and discrete photoconductive particles, said colored toner particles substantially lacking the property of photoconductivity and comprising a colorant selected from the group consisting of a pigment and a dye having a thin layer of a resin absorbed therearound, said photoconductive particles comprising particulate photoconductive material having a thin layer of a resin absorbed therearound, said thin layer of said resin absorbed therearound said particulate photoconductive material being sufficiently thin to facilitate exposure of said particulate photoconductive material and dissipate any charge thereon; said photoconductive particles being present in an amount of from about 5 to about 104 parts by weight for every 100 parts by weight of said colored toner particles;

h. contacting said photoconductive insulating layer with an insulating liquid other than the developer liquid to neutralize any residual charge in the portion of said layer developed in step (g);

i. charging said photoconductive insulating layer;

j. exposing the charged layer to said original colored object through a colored filter to form a third primary color coded electrostatic latent image on said layer; and

k. developing said third electrostatic latent image with a liquid developer having a color complementary to said third color coded image, said liquid developer comprising an insulating liquid having dispersed therein colored particles.

2. The method of claim 1 wherein said photoconductive particles are dye sensitized.

3. The method of claim 1 wherein said photoconductive particles are zinc oxide.

4. The method of claim 1 wherein said colorant is an organic dye which is substantially insoluble in said carrier liquid.

5. The method of claim 1 wherein said photoconductive particles contain less than about 2 parts by weight of said resin per 100 parts of said particulate photoconductive material.

6. The method of claim 1 wherein said photoconductive particles have a particle size of from about 0.1 to about 1.0 micron.

7. The method of claim 1 wherein said colored toner particles have a particle size of from about 0.01 to about 0.5 micron.

8. The method of producing a reproduction of a colored object comprising the steps of:

- a. charging a photoconductive insulating layer;
- b. exposing said layer to a wavelength of light corresponding to a primary color to produce an electrostatic latent image;
- c. developing said electrostatic latent image with a liquid developer comprising an insulating liquid having a dielectric constant of less than about 3.4 and a volume resistivity of greater than about  $10^{10}$  ohm-cm so as not to affect an electrostatic latent image formed on said insulating layer, and dispersed therein a mixture of discrete photoconductive particles and discrete toner particles complementary to the radiation of exposure in step (b); said colored toner particles substantially lacking the property of photoconductivity and comprising

a colorant selected from the group consisting of a pigment and a dye having a thin layer of a resin absorbed therearound, said photoconductive particles comprising particulate photoconductive material having a thin layer of a resin absorbed therearound, said thin layer of said resin absorbed therearound said particulate photoconductive material being sufficiently thin to facilitate exposure to said particulate photoconductive material and dissipate any charge thereon, said photoconductive particles being present in an amount of from about 5 to about 104 parts by weight for every 100 parts by weight of said colored toner particles;

10

d. contacting said photoconductive insulating layer with an insulating liquid other than the developer liquid to neutralize any residual charge in the portion of said layer developed in step (c);

e. charging said photoconductive insulating layer;

f. exposing said layer to a wavelength of light corresponding to a primary color different from that of step (b) to produce an electrostatic latent image;

20

g. developing said electrostatic latent image with a liquid developer as in step (c) wherein said liquid developer particles are complementary to the radiation of exposure in step (f);

25

h. contacting said photoconductive insulating layer with an insulating liquid other than the developer liquid to neutralize any residual charge in the portion of said layer developed in step (g);

30

i. charging said photoconductive insulating layer;

j. exposing said layer to a wavelength of light corresponding to a primary color different from that of steps (b) and (f) to produce an electrostatic latent image; and

35

k. developing said electrostatic latent image with a liquid developer as in step (c) wherein said liquid developer particles are complementary to the radiation of exposure in step (j).

9. The method of claim 8 wherein said photoconductive particles are dye sensitized.

14

10. The method of claim 8 wherein said photoconductive particles are zinc oxide.

11. The method of producing a reproduction of a colored object comprising the steps of:

a. charging a photoconductive insulating layer;

b. exposing said layer to a wavelength of light corresponding to a color to produce an electrostatic latent image;

c. developing said electrostatic latent image with a liquid developer comprising a carrier liquid having a dielectric constant of less than about 3.4 and a volume resistivity of greater than about  $10^{10}$  ohm-cm so as not to affect an electrostatic latent image formed on an insulating layer, and dispersed in said carrier liquid, a mixture of discrete colored toner particles and discrete photoconductive particles, said colored toner particles substantially lacking the property of photoconductivity and comprising a colorant selected from the group consisting of a pigment and a dye having a thin layer of a resin absorbed therearound, said photoconductive particles comprising particulate photoconductive material having a thin layer of a resin absorbed therearound, said thin layer of said resin absorbed therearound said particulate photoconductive material being sufficiently thin to facilitate exposure of said particulate photoconductive material and dissipate any charge thereon, said photoconductive particles being present in an amount of from about 5 to about 104 parts by weight for every 100 parts by weight of said colored toner particles, said toner particles being complementary to the radiation of exposure in step (b);

d. contacting said photoconductive insulating layer with an insulating liquid other than the developer liquid to neutralize any residual charge in the portion of said layer developed in (c); and

e. repeating steps (a), (b), (c), and (d) at least one additional time wherein the wavelength of light in the exposure step is other than that of step (b).

\* \* \* \* \*